

H. L. & E. A. SULMAN.  
ORE CONCENTRATOR.  
APPLICATION FILED JULY 31, 1906.

902,018.

Patented Oct. 27, 1908.



Witnesses.  
H. Totten  
M. G. Lockett.

Inventors  
Henry L. Sulman  
Evan Aspray Sulman  
By Knight & Co  
Attorneys

# UNITED STATES PATENT OFFICE.

HENRY LIVINGSTONE SULMAN AND EVAN ASPRAY SULMAN, OF LONDON, ENGLAND,  
ASSIGNORS TO MINERALS SEPARATION, LIMITED, OF LONDON, ENGLAND.

## ORE-CONCENTRATOR.

No. 902,018.

Specification of Letters Patent.

Patented Oct. 27, 1908.

Application filed July 31, 1906. Serial No. 328,551.

*To all whom it may concern:*

Be it known that we, HENRY LIVINGSTONE SULMAN and EVAN ASPRAY SULMAN, subjects of the King of England, residing at 5 London, England, and Highgate, London, England, respectively, have invented a certain new and useful Ore-Concentrator, of which the following is a specification.

This invention relates to improvements in 10 ore concentrators, the object being to provide suitable means for separating metalliferous particles from gangue or from one another.

Hitherto it has been proposed to separate mineral particles which are immersed in liquid by causing the particles to be exposed to the air and thereafter to meet the edge or surface of liquid, whereby certain particles float and are separated from the remainder. In the apparatus previously suggested, the 15 powdered ore was carried on some form of moving surface, such as a vanning table or conveyer.

An ore concentrator according to this invention comprises a fixed surface over which 20 the powdered ore and a thin layer of liquid are fed, and means for alternately exposing the ore to the air and to the edge of the liquid whereby certain particles are caused to float, and are separated from the remainder.

30 The apparatus may consist of a fixed inclined surface over which powdered ore will not flow, means for distributing a thin stream of liquid over the surface, means for supplying powdered ore to the surface, a 35 movable body having a flexible edge in contact with the surface, means for sweeping the body over the surface to remove the layer of liquid temporarily from the ore and also to feed the ore over the surface and means for 40 collecting the floating and immersed materials which are discharged from the surface.

In a preferred form of the apparatus the 45 surface on which separation takes place is a flat conical buddle having a smooth surface, conveniently of rubber. A vertical shaft is rotated at the center of the buddle and a receptacle for powdered ore is carried on the shaft and a conduit from said receptacle feeds the powdered ore on to the buddle.

50 Perforated liquid-distributing pipes radiate from the shaft; liquid is supplied to the pipes by any suitable means and a thin stream of liquid is thus produced over the buddle. Arms radiating from the shaft, and preferably in the form of volutes, have rubber

edges in contact with the surface to remove the layer of liquid temporarily from the ore and also to feed the ore over the buddle. The periphery of the buddle dips into a launder which receives the material discharged 60 from its surface and a second launder is arranged to receive the overflow from the first launder carrying the floating material.

The accompanying drawing is a perspective view, partly in section, of one form of 65 apparatus embodying this invention.

A conical buddle A is inclined at a small angle, say one in twenty, such that the ore will not flow over it of its own accord and the buddle may conveniently be covered with 70 india rubber, wood, or other smooth material.

A rotatable vertical shaft B passes through the center of the buddle, is supported in suitable bearings B<sup>1</sup> and is driven by suitable 75 gear B<sup>2</sup>. A receptacle C for the ore may be carried on the shaft, and conduits C<sup>1</sup> convey the ore from the receptacle C on to the buddle A. Liquid-distributing pipes D, which may be straight or curved, radiate from the 80 shaft B. Liquid such as acidified water is supplied to these pipes through a suitable conduit D<sup>1</sup> and the pipes are perforated, as at D<sup>2</sup>, so as to distribute a thin layer of liquid over the buddle. Arms E, preferably in the 85 form of volutes, radiate from the shaft B and have flexible edges or squeegees E<sup>1</sup> in contact with the surface of the buddle. By "squeegee" we mean a flexible edge such as rubber which is capable while being moved 90 over a slightly uneven surface of adapting itself to that surface and of removing water therefrom. The periphery of the buddle dips into an annular launder F into which the solid particles which remain on the surface of the buddle are discharged. A second 95 launder G is arranged to receive the surface water from the buddle carrying the floating material which is thereby separated from the material which does not float.

The operation of the apparatus is as follows:—Powdered ore, conveniently in the form of thick pulp, is fed from the receptacle C through the pipes C<sup>1</sup> on to the buddle A near the center and is spread out over the surface of the buddle by the rotating arms E. The distributing pipes D cause a thin layer of liquid to flow over the surface of the buddle towards its periphery. As the arms E, carrying the squeegees E<sup>1</sup> of india rubber or 110

other flexible material, pass over the surface of the bundle, the solid matter is partly pushed forward by the arms and therefore caused to pass towards the circumference of 5 the bundle, and at the same time the squeegees pass over the particles, temporarily removing the liquid therefrom, so that the particles are exposed to the air. The layer of liquid from the distributors D then passes 10 over the surface again and, as the oncoming film of liquid meets the particles, certain of these are caused to float and remain floating on the liquid after it has passed over the bundle. The material which remains on the 15 surface of the bundle is gradually fed outwards and sinks into the launder F at the periphery, while the particles which float on the liquid pass over the edge of the first launder into the second launder G and are 20 thence collected.

The apparatus has been described in one preferred form; but it is to be understood that the details of arrangement and construction may be varied without departing 25 from this invention.

What we claim as our invention and desire to secure by Letters Patent is:—

1. In an apparatus for concentrating ores the combination of a fixed surface, means 30 for feeding powdered ore over the surface, means for continuously feeding a thin stream of liquid over the surface, a movable body having a flexible squeegee edge in contact with the surface sufficiently flexible to pass 35 over the ore while exerting sufficient pressure on the surface to remove the film of water therefrom, means for sweeping the body over the surface in a direction at right angles to the direction of flow of the water to cause the 40 ore to be alternately exposed to the air and to the edge of the liquid.

2. In an apparatus for concentrating ores the combination of a fixed inclined surface over which powdered ore will not flow, 45 means for continuously distributing a thin stream of liquid over the surface, means for supplying powdered ore to the surface, a movable body having a flexible squeegee edge in contact with the surface sufficiently 50 flexible to pass over the ore while exerting sufficient pressure on the surface to remove the film of water therefrom, means for sweeping the body over the surface in a direction at right angles to the direction of 55 flow of the water to remove the layer of liquid temporarily from the ore and also to feed the ore over the surface.

3. In an apparatus for concentrating ores the combination of a fixed inclined surface 60 over which powdered ore will not flow, means for continuously distributing a thin stream of liquid over the surface, means for supplying powdered ore to the surface, a movable body having a flexible squeegee 65 edge in contact with the surface sufficiently

flexible to pass over the ore while exerting sufficient pressure on the surface to remove the film of water therefrom, means for sweeping the body over the surface in a direction at right angles to the direction of flow of the 70 water to remove the layer of liquid temporarily from the ore and also to feed the ore over the surface, means for collecting the floating material from the surface, and means for collecting the discharged material which 75 does not float.

4. In an apparatus for concentrating ores the combination with a fixed inclined surface over which powdered ore and a thin layer of liquid are continuously fed of a squeegee sufficiently flexible to pass over the ore while exerting sufficient pressure on the surface to remove the film of water therefrom which is swept over the surface intermittently in a direction at right angles to the direction of 85 flow of the water to remove the layer of liquid from the ore, whereby the ore is alternately exposed to the air and to the advancing edge of the layer of liquid.

5. In an ore concentrator the combination 90 of a fixed conical surface of wide angle at the apex, means for continuously distributing a thin stream of liquid over the surface, means for supplying powdered ore to the surface, a movable arm having a flexible squeegee edge 95 in contact with the surface sufficiently flexible to pass over the ore while exerting sufficient pressure on the surface to remove the film of water therefrom, means for sweeping the arm over the surface in a direction at 100 right angles to the direction of flow of the water to remove the layer of liquid temporarily from the ore and to feed the ore over the surface, means for collecting the floating material from the surface and means for collecting the discharged material which does 105 not float.

6. In an ore concentrator the combination of a fixed conical surface of wide angle at the apex, a rotatable vertical shaft at the center 110 thereof, means for rotating the shaft, means for supplying powdered ore on to the bundle, a perforated liquid-distributing pipe radiating from the shaft, and means for supplying liquid continuously thereto to produce a 1 thin stream of liquid over the bundle, arms 115 radiating from the shaft, flexible squeegee edges on the arms sufficiently flexible to pass over the ore while exerting sufficient pressure on the surface to remove the film of 120 water therefrom in contact with the surface to remove the layer of liquid temporarily from the ore and to feed the ore over the bundle, means for collecting the floating material discharged from the bundle and means 125 for collecting the discharged material which does not float.

7. In an ore concentrator the combination of a fixed conical surface of wide angle at the apex, a rotatable vertical shaft at the center 130

thereof, means for rotating the shatt, a receptacle for powdered ore carried on the shaft, a conduit from said receptacle to feed powdered ore on to the buddle, perforated liquid-distributing pipes radiating from the shaft and means for supplying liquid continuously thereto to produce a thin stream of liquid over the buddle, volute arms radiating from the shaft, flexible squeegee edges on the 5 arms sufficiently flexible to pass over the ore while exerting sufficient pressure on the surface to remove the film of water therefrom in contact with the surface to remove the layer of liquid temporarily from the ore and 10 to feed the ore over the buddle, means for collecting the floating material discharged from the buddle and means for collecting the 15 discharged material which does not float.

8. In an ore concentrator the combination 20 of a fixed conical surface of wide angle at the apex, a rotatable vertical shaft at the center thereof, means for rotating the shaft, a receptacle for powdered ore carried on the shaft, a conduit from said receptacle to feed powdered ore on to the buddle, perforated liquid-distributing pipes radiating from the shaft, and means for supplying liquid continuously thereto to produce a thin stream of liquid over the buddle, volute arms radiating 25 from the shaft, flexible squeegee edges on the arms sufficiently flexible to pass over the ore while exerting sufficient pressure on the surface to remove the film of water therefrom in contact with the surface to remove the 30 layer of liquid temporarily from the ore and to feed the ore over the buddle, a first laun- 35

der at the periphery of the buddle to receive the material discharged from its surface, and a second launder arranged to receive the overflow carrying the floating material.

9. In an ore concentrator the combination 40 of a fixed conical surface of wide angle at the apex and covered with rubber, a rotatable vertical shaft at the center, means for rotating the shaft, a receptacle for powdered ore carried on the shaft, a conduit from said receptacle to feed the powdered ore on to the buddle, perforated liquid-distributing pipes radiating from the shaft and means for supplying liquid continuously thereto to pro- 45

50

55

60

65

duce a thin stream of liquid over the buddle, volute arms radiating from the shaft, rubber squeegee edges on the arms sufficiently flexible to pass over the ore while exerting sufficient pressure on the surface to remove the film of water therefrom in contact with the surface to remove the layer of liquid temporarily from the ore and to feed the ore over the buddle, a first launder at the periphery of the buddle to receive the material discharged from its surface and a second launder arranged to receive the overflow from the first launder carrying floating material.

In testimony whereof we have signed our names to this specification in the presence of 65 two subscribing witnesses.

HENRY LIVINGSTONE SULMAN  
EVAN ASPRAY SULMAN.

Witnesses:

ALBERT OWEN WILLIAMS,  
WILLIAM H. BALLANTYNE.